

## UNITED STATES PATENT OFFICE

2,215,563

## PROCESS FOR COATING FABRICS WITH RUBBER

Stewart R. Ogilby, Staten Island, N. Y., assignor to United States Rubber Company, New York, N. Y., a corporation of New Jersey

No Drawing. Application April 7, 1939,  
Serial No. 266,535

## 6 Claims. (Cl. 28—1)

This invention relates to a process for coating fabrics with rubber, and more particularly for coating fabrics directly from latex.

In coating fabrics directly from latex, it is very desirable to use a heat sensitive latex composition so that on raising the temperature of the latex after spreading, as in the early stages of a drying operation, the latex will set to a gel and prevent "striking through" of the latex and the consequent marring of the appearance of the untreated surface of the fabric. In producing dyed fabrics having a rubber coating thereon, it is often desirable and in some cases necessary to apply the rubber to the fabric before the dyeing operation. Commonly, latex compositions which have been so compounded as to be capable of gelling on heating are alkaline in character and leave a final rubber deposit on the fabric having an alkaline reaction. Dye baths for fabrics are often neutral or slightly acid and when a fabric coated with rubber which has an alkaline reaction is introduced into such a dye bath, the alkaline reaction of the rubber may oftentimes change the pH of the bath sufficiently to give off-colors in the final dyed fabric.

According to the present invention, fabrics may be coated with a latex composition which is heat sensitive and which has an acid reaction so that on the gelling, or the gelling and drying, of such a latex composition on a fabric, the deposit will have an acid or neutral character and hence not detrimentally affect the color of the dyed material by raising the pH, as in the case of a rubber deposit having an alkaline reaction.

I have found that a latex composition stabilized by the addition to the latex of a condensation product of a straight chain aliphatic alcohol having at least six carbon atoms with a polyglycol compound containing at least four ethenoxy groups may be made heat sensitive by adjusting its pH to below 7. The commercial name of one of such commercial products is "Emulphor-O," believed to be the condensation product of tetraethylene glycol with oleyl alcohol. It has been found that up to 5% of "Emulphor-O," for example, permits a latex composition of over 30% solids content to be acidified as far as a pH of 1, and yet the "Emulphor-O" will lose its power to protect the latex at elevated temperatures and the latex composition will gel on heating.

The present invention may be utilized in the manufacture of various types of fabrics, some or all of whose threads or yarns are to be dyed after coating with the latex composition. In

these cases, there is no residual alkalinity in the latex gel, or the dried rubber deposit to produce off-colors in the dyeing operation. The present invention may also be applied to the coating of fabrics where the fabrics are not to be dyed after coating, but where it is desired that the spread latex or the final rubber coating have an acid or neutral reaction. If the pH of the latex, according to the present invention, is lowered below 7 by the addition of a volatile acid, then the latex after gelling will retain an acid reaction, but on drying the rubber deposit will be neutral.

The present invention is of particular advantage in the manufacture of pile fabrics where the pile is looped around threads in a woven textile

backing and the piles are anchored to the backing by means of a rubber coating or deposit.

Such pile fabrics are commonly woven on the so-called double plush principle, where two textile backings or ground fabrics are woven with pile

warps looped around weft threads in each backing and where the piles are cut intermediate the two backings to produce two pile fabrics. In upholstered fabrics of such construction, the textile

backing is usually woven of cotton yarns and these, if desired, may be predyed before weaving.

The pile warps are commonly animal hair and these are generally dyed after the woven and split fabrics have been treated with latex according to the present invention. In carrying out

the present invention with reference to such pile fabrics, the heat sensitive latex having a pH below 7 and capable of gelling at an elevated temperature, is spread onto the back of the pile fabric as by means of a spreader knife or by spray-

ing or in any desired manner. Only sufficient latex need be applied to satisfactorily anchor the piles to the ground fabric after drying of the rubber film.

The latex may be scraped onto the back of the pile fabric in such a manner that the tips of the pile bights will project from the final rubber coating, as in the present practice of making this type of upholstery fabrics. After spreading the latex compound, the deposit is heated to a temperature sufficient to gel the latex

whereby striking-through of the latex on further treatment is prevented. In that the latex will not strike through after gelling, the gelled latex need not be dried before subsequent aqueous treatments.

It is preferred, however, to dry the fabric before dyeing and finishing, and in such case the fabric need only be passed into a drier after being spread with latex and the gelling will take place in the first stages of the drying operation where, as is generally the case, the tem-

5  
5  
10  
15  
20  
25  
30  
35  
40  
45  
50  
55

perature of the entrance to the drier is above the gelling temperature of the latex composition. The thus coated fabric may then be dyed in the usual manner without the pH of the dye bath being raised by the rubber deposit. Where the textile backing or ground fabric and the piles are of two different kinds of fibers, the dye bath may be prepared so as to dye only the pile or, as in the case of the ground fabric and pile being composed of the same kind of fibers, the dye bath may dye both the piles and the ground fabric.

The following formula is illustrative of a latex composition which may be used for anchoring mohair piles to a cotton ground fabric in a pile fabric woven on the double plush principle:

| Parts by weight                       |                 |     |
|---------------------------------------|-----------------|-----|
| Latex                                 | Rubber          | 100 |
|                                       | Water           | 62  |
| 20                                    | NH <sub>3</sub> | .2  |
| 25 % aqueous solution of "Emulphor-O" |                 | 12  |
| 15 % aqueous solution of acetic acid  |                 | 25  |

The above latex compound has a pH of 4.4 and a dried rubber film deposited from it has a neutral reaction due to the volatilization of the acetic acid on drying. This latex is fluid at ordinary room temperatures and will gel at temperatures of 85° C. or above. It is thus only necessary to spread the latex compound on the back 30 of the pile fabric at temperatures below the gelling temperature, and after spreading to pass the spread fabric through a conventional drier having a temperature greater than 85° C. at its entrance so that the latex compound will gel in 35 the first stages of the drying operation, and the further heating of the gel to dry the same will evaporate water from the gel without the rubber particles which are no longer mobile striking through and marring the face of the fabric. Various other compounds may be used, and 40 the latex may be unvulcanized or vulcanized as desired.

In view of the many changes and modifications that may be made without departing from the principles underlying the invention, reference should be made to the appended claims for an understanding of the scope of the invention.

Having thus described my invention, what I claim and desire to protect by Letters Patent is:

1. The process of coating a fabric with rubber which comprises applying to a fabric a fluid latex composition having a pH below 7 and containing a condensation product of a straight chain aliphatic alcohol having at least six carbon atoms with a polyglycol compound containing at least four ethenoxy groups, said latex composition being fluid at room temperature and

capable of gelling at elevated temperature, heating the applied latex composition to a temperature sufficient to gel the same, and drying.

2. The process of coating a fabric with rubber which comprises applying to a fabric a fluid latex composition having a pH below 7 and containing "Emulphor-O", said latex composition being fluid at room temperature and capable of gelling at elevated temperature, heating the applied latex composition to a temperature sufficient to gel the same, and drying.

3. The process of producing a dyed fabric with a rubber coating thereon which comprises applying to an undyed fabric a fluid latex composition having a pH below 7, and containing a condensation product of a straight chain aliphatic alcohol having at least six carbon atoms with a polyglycol compound containing at least four ethenoxy groups, said latex composition being fluid at room temperature and capable of gelling at elevated temperature, heating the applied latex composition to a temperature sufficient to gel the same, and dyeing the coated fabric.

4. The process of producing a dyed fabric with a rubber coating thereon which comprises applying to an undyed fabric a fluid latex composition having a pH below 7 and containing "Emulphor-O," said latex composition being fluid at room temperature and capable of gelling at elevated temperature, heating the applied latex composition to a temperature sufficient to gel the same, and dyeing the coated fabric.

5. The process of making pile fabric which comprises weaving a textile backing with undyed pile warps looped therein, applying to the backing and pile loops a fluid latex composition having a pH below 7 and containing a condensation product of a straight chain aliphatic alcohol having at least six carbon atoms with a polyglycol compound containing at least four ethenoxy groups, said latex composition being fluid at room temperature and capable of gelling at elevated temperature, heating the applied latex composition to a temperature sufficient to gel the same, and dyeing the coated fabric.

6. The process of making pile fabric which comprises weaving a textile backing with undyed pile warps looped therein, applying to the backing and pile loops a fluid latex composition having a pH below 7 and containing "Emulphor-O," said latex composition being fluid at room temperature and capable of gelling at elevated temperature, heating the applied latex composition to a temperature sufficient to gel the same, and dyeing the coated fabric.

STEWART R. OGILBY.